

## UNITED STATES PATENT OFFICE

BENNO BORZYKOWSKI, OF PARIS, FRANCE, ASSIGNOR TO SWISS BORVISK COMPANY,  
OF WILMINGTON, DELAWARE, A CORPORATION OF DELAWARE

## ARTIFICIAL SILK AND THE PROCESS OF PRODUCING THE SAME

No Drawing. Application filed September 27, 1926, Serial No. 138,122, and in Germany November 11, 1925.

In the artificial silk industry, particularly at the beginning of this branch of the art, great importance was attached to the production of fibres having a very brilliant lustre.

5 During the course of time, however, as the field of use of artificial silk greatly increased, a demand arose for fibres not having this very brilliant lustre, but having a duller, or silk-like aspect. Many proposals have been  
10 made for securing this result.

I have now found it possible to produce utilizable dull finish fibres with a silk-like lustre by producing the fibres in known manner from viscose, but with a subsequent treatment  
15 which forms the essential feature of the present invention.

The setting of the thread from the viscose solution can be effected in known manner, by the use of any of the commonly used setting baths. The viscose used can be of any age (or stage of ripeness), or can be fresh  
20 (i. e. directly after its original preparation). As is known, in the said operation a part of the sulfur is set free, during the setting operation, in a very finely divided state, perhaps colloidal, on the surface of (and to some extent within) the threads or filaments. This may exist as elemental sulfur, or as precipitated sulfur-containing by-products, in  
25 soluble in water but existing in a very finely divided state.

In my process, the silk is not, as is usually done, desulfurized before the bleaching, but  
30 (after washing out soluble acids and salts, if desired) may be bleached directly with the adherent sulfur. The result thereof is that colloidal precipitates or deposits are formed which are not removed or are only partially removed, during subsequent washing.

40 The dull, silk-like appearance of the fibre obtained in this manner is permanent and does not disappear even when the artificial silk is dyed.

The action of the adhering salts for the  
45 formation of colloidal precipitations or depositions, on or in the silk fibres, may be further increased by passage of the raw artificial silk through a suitable salt solution before the reviving (scooping, or toning), operation.

*Example.*—Viscose silk prepared in the usual or any approved manner, but without being subjected to the usual desulfurizing operation, is subjected to the usual washing and twisting, is preferably formed into 55 hanks or skeins and then, as so-called raw silk, it may be introduced directly (that is, without being preliminarily desulfurized), into a bleaching bath containing, for example, 60 0.01 to 0.15% of free chlorine. The bleaching may be performed with other bleaching agents that do not dissolve elemental sulfur, e. g.  $H_2O_2$ , or numerous others. In some cases, as where the silk is to be dyed a dark color, the bleaching operation may be omitted. 65 It is then passed (if it has been treated with chlorine) into an acid bath, to which aluminum, magnesium, zinc or other similar salts (say sulfates or chlorides) may be added. The salts of these metals are of especial interest because the salts themselves and any insoluble compounds thereof, formed in the process, are white, and hence do not discolor the silk. The amount of salts is (in said bath, or a separate bath if acid is not used) 70 preferably from 1 to 2% with respect to the bath. As is known, one effect of the salts in this bath, is to prevent excessive action of the acid of this bath upon the silk, and in the present instance the salts in this 75 bath react with the undesulfurized fibre to form white colloidal precipitations upon or in the silk fibres.

The silk is then treated in the usual toning (scooping) bath (say soap solution) until 80 the silk skein just shows a weakly acid reaction.

## I claim:

1. In the production of dull finish viscose silk, the herein described improvement of 85 treating the viscose silk, while still containing sulphur, directly with a bleaching agent which will not remove such sulphur.

2. A process of producing artificial silk with a dull silk-like luster and appearance, 90 which comprises treating raw viscose silk, with a solution of an earth metal salt capable of producing a substantially colloidal precipitate upon and in the fibres of the silk, and thereafter toning (scooping) in the 95 100

usual manner, all without subjecting said silk to a desulfurizing treatment.

3. Finished viscose silk retaining its original substantially colloidally precipitated sulphur and having a white earth metal compound precipitated in a substantially colloidal state on and in its fibres, the same having a dull silk-like lustre which is persistent even after dyeing.

10 4. A process which comprises forming upon the fibres of undesulfurized viscose silk, a very finely divided precipitate, from a soluble earth-metal salt, to thereby give a dull silk-like effect to the product.

15 5. Bleached viscose silk retaining its original colloidally precipitated sulphur, in a substantially colloidal state, on and in its fibres, the same having a dull silk-like lustre which is persistent even after dyeing.

20 In testimony whereof I have signed my name to this specification.

BENNO BORZYKOWSKI.

25

30

35

40

45

50

55

60